

# UNITED STATES PATENT OFFICE.

NOAK VICTOR HYBINETTE, OF CHRISTIANIA, NORWAY, ASSIGNOR TO PACIFIC SECURITIES COMPANY LIMITED, OF TORONTO, CANADA.

## ANODE FOR ELECTROLYSIS.

1,128,316.

Specification of Letters Patent.

Patented Feb. 16, 1915.

No Drawing. Original application filed June 5, 1912, Serial No. 701,780. Divided and this application filed June 26, 1913. Serial No. 775,956.

*To all whom it may concern:*

Be it known that I, NOAK VICTOR HYBINETTE, a subject of the King of Norway, residing at Christiania, Norway, have invented Improvements in Anodes for Electrolysis, of which the following is a specification, and is a division of my application, Serial No. 701,780, filed June 5, 1912.

This invention has for its object a process 10 of separating copper from nickel.

In a patent granted to me in U. S. A. November 28th 1905 under No. 805,969, I describe a process of refining copper-nickel matte. The matte is roasted and eventually leached to remove a possible excess of copper and the roasted material, whether leached or not, is smelted and cast into anodes or metallic slabs. The anodes are electrolyzed in acid nickel sulfate solution, 20 whereupon copper is cemented out from the electrolyzed solution upon metallic slabs. My patent above referred to, prescribes that at least part of the material should be free from carbon, silicon and sulfur.

I have found that it is entirely too expensive to reduce, smelt and cast a slab practically free from sulfur, carbon and silicon, as proposed in my patent above referred to. I have found that smelting of 30 such an anode is only possible in a reverberatory furnace and in such a furnace the reduction of oxid to metal is hard to accomplish. On the other hand such reduction is made automatically by blast furnace smelting. The alloy of 3 parts nickel and 1 part copper is however too hard to be smelted in a blast furnace and cast into anode slabs directly from the furnace. To accomplish this, I introduce about 4-8 % sulfur in the 40 anode which is added to the roasted and leached matte in the shape of unroasted matte. In case the proportion of copper is low in the raw material no leaching is done and an incomplete roasting leaves the necessary sulfur in the material.

The cementation of copper from the electrolyte is under ordinary conditions impracticable with a metal slab containing 4-8 % sulfur. Even when using a copper nickel 50 alloy free from sulfur carbon and silicon (as in my old patent above referred to), I preferred to carry out the last part of the

cementation on pure nickel. I have now found that the cementation is possible and can be carried to completion in one operation by the use of slabs containing 4-8 % sulfur, that is slabs cast from a blast furnace and of the same composition as the anodes, provided, that these slabs have been previously used as anodes in a nickel plating tank and thereby the surface prepared in such a way that the cementation will take place. Why the cementation will take place under these conditions and not on a fresh cast surface depends probably thereupon 55 that when a fresh surface is subjected to cementation there is formed a coherent sheet of metallic copper which partly at least prevents further cementation, whereas a surface previously used as anode in an electrolytic 60 bath has a porous surface covered by slimes of metal and sulfids whereby the copper is cemented on top of these slimes and comes down as a spongy mass through which the solution can percolate. The spongy mass on 65 the surface stands in metallic contact with the solid part of the slab and may also be said to help the cementation simply by the larger surface which it presents.

What I claim is:

1. An anode for the cementation of copper, which consists mainly of nickel, copper and sulfur, the sulfur content being high, said anode having an electrolytically treated surface.

2. An anode for the cementation of copper, which consists mainly of nickel, copper and between four and eight per cent. sulfur, and has an electrolytically treated surface.

3. The method of making anodes for copper cementation, which comprises subjecting a charge of copper nickel matte containing sulfur to the reducing action of a blast in a suitable furnace, and proportioning said charge to obtain a product containing from four to eight per cent. of sulfur, casting the product into slabs and surface treating the slabs by electrolysis.

Signed at London, England, this 9th day of June 1913.

NOAK VICTOR HYBINETTE.

Witnesses:

H. D. JAMESON,  
O. J. WORTH.